

## 1

3,630,856

**ELECTRODEPOSITION OF RUTHENIUM**  
Andre Meyer, Geneva, Switzerland, assignor to Sel-Rex  
Corporation, Nutley, N.J.

No Drawing. Filed Mar. 20, 1970, Ser. No. 21,533  
Claims priority, application Switzerland, Mar. 21, 1969,  
4,277/69

U.S. CL. 204—43

Int. CL. C23b 5/32

2 Claims

### ABSTRACT OF THE DISCLOSURE

Thick electrodeposits of ruthenium can be obtained by adding an element selected from gallium, indium, and thallium in a stable and soluble form. The deposits obtained are primarily characterized by their low stress and absence of surface cracks at thicknesses up to about 10 millimicrons.

The present invention relates to a method for the electrodeposition of ruthenium and to an aqueous bath for carrying out this method.

It is known to electrolytically produce ruthenium coatings by using, as an electrolyte, a complex having the formula  $(\text{NH}_4)_3[\text{Ru}_2\text{Cl}_8(\text{H}_2\text{O})_2\text{N}]$ , containing 34.4% in weight of ruthenium metal, at several current densities.

The ruthenium coatings so obtained are characterized by severe inner stress, so that they show cracks when their thickness is above 1.0 to 1.5  $\mu\text{m}$ . Today most commercial applications of parts plated with ruthenium require substantially thicker coatings, usually of the order of a minimum thickness of 2.5  $\mu\text{m}$ . to 5  $\mu\text{m}$ . or even, on occasion, somewhat thicker, up to about 10  $\mu\text{m}$ .

The object of the present invention is to permit the electrodeposition of ruthenium coatings of a thickness sufficient to meet contemporary industrial needs. In particular, it is an object of the present invention to permit the production of ruthenium coatings of a thickness of up to about 10  $\mu\text{m}$ . while comprising no visible cracks even at a magnification of 500 times.

This invention is based on the discovery that the addition of one of the elements selected from gallium, indium and thallium in the form of a stable, soluble compound to a ruthenium plating solution, serves to severely reduce inner surface stress of the plated ruthenium to the point where relatively thick deposits of ruthenium electroplate can be obtained. In general, one of the elements selected from gallium, indium and thallium is added in concentration from 50 mg./l. up to saturation to an aqueous solution of a ruthenium compound which contains from about 0.5 g./l. to about 50 g./l. of ruthenium metal.

The addition of at least one metal selected from gallium, indium and thallium, as stable and water soluble compounds, results in coatings which are more ductile. These metallic compounds which appear in the cathodic film during the electrolysis modify the cathodic polarization and the crystallization phenomena, and produce coatings which are completely different from those heretofore obtained by known methods, in their appearance (brighter and clearer), in their mechanical characteristics (more ductile, without cracks), and in their composition, the metals of addition being co-deposited with the ruthenium during the electrolysis. Some secondary effects due to the addition of these metals have also been found, especially a slight improvement of the cathodic efficiency, almost at high current density, and a higher power of macro and micro-repartition.

## 2

### EXAMPLES

(1) A bath has been prepared containing:

Ruthenium: 10 g./l. as a complex of



containing 34.4% in weight of ruthenium metal

Indium: 5 g./l. (as sulfate)

Ammonium sulfamate: 15 g./l. (conductivity salt)

pH adjusted to 1.5 by means of  $\text{NH}_4\text{OH}$  or  $\text{HCl}$  or  $\text{H}_2\text{SO}_4$

Temperature of the bath: 60° C.

Current density: 1 amp. $\text{dm}^2$

The light coatings, produced on samples of brass precoated with a flash of gold, showing no visible cracks or micro-cracks, to thicknesses up to about 10  $\mu\text{m}$ ., have been obtained at a plating rate of 12 mg./amp.min., that represent 1  $\mu\text{m}$ . in 9 minutes. These deposits contained about 1.2 to 1.5% indium.

(2) Deposits have been effected by means of the following bath:

Ruthenium: 10 g./l. as a complex of



Indium: 3 g./l. (as sulfamate)

Ammonium sulfamate: 5 g./l.

Sulphamic acid: 5 g./l.

Sulfuric acid up to a pH of 1.0 to 1.5

Temperature of bath: 65 to 70° C.

Current density: 1 amp. $\text{dm}^2$

Bright coatings of ruthenium were obtained on brass samples precoated with a flash of gold which showed no visible cracks or micro-cracks, and for this thicknesses up to 10  $\mu\text{m}$ . These coatings were obtained at a plating rate of 11 mg./amp.min. These deposits contained about 1.0 to 1.3% indium.

Along with the deposit of ruthenium there will be a co-deposit of the Group III-B metal chosen. That codeposit will generally be on the order of about 0.1% to 10.0% of the total content of the electrodeposit. At about 5 g./l. of a Group III-B metal, the metal will codeposit with ruthenium in a range of about 1.0 to 2.0%.

The above examples have only an illustrative purpose and are not to be considered, in any way, as being limitative.

Experience has shown that indium and gallium give the best result, thallium being less soluble and presenting a tendency to crystallize partially.

The effects of the addition are substantial from a concentration of about 100 mg./l. the maximum effect being obtained, however, with an addition of 5 g./l. of indium, for instance. Above this concentration, no substantial supplementary effect appears.

At pH higher than 1.5, the deposits obtained are less bright and have a greater tendency to present micro-cracks and pits which alter its appearance.

The cathodic efficiency increases with the temperature. Between 60 and 80° it is practically constant. On the other hand, it shows a tendency to decrease while the current density increases.

The plating can be effected on any support permitting an electrodeposition, especially on the same supports as those which permit the coating of gold, like brass, nickel, titanium, etc.

So as to produce a better adherence and for limiting the formation of porous deposits, it is advantageous, in some cases, to apply on the support, before the electrodeposition of ruthenium, a flash of gold.

I claim:

1. A method for electrodepositing ruthenium by passing a current through an aqueous solution containing from about 0.5 g./l. to about 50 g./l. of ruthenium and at least one element selected from the group consisting of gallium, indium and thallium in a stable and soluble form and in a concentration from about 50 mg./l. up to saturation, whereby ruthenium is deposited on the cathode.

2. An aqueous electroplating solution containing from about 0.5 g./l. to about 50 g./l. of ruthenium and at least 10 one element selected from the group consisting of gallium,

indium, and thallium in a stable and soluble form and in a concentration from about 50 mg./l. to saturation.

**References Cited**

5      Frederick A. Lowenheim: Modern Electroplating, p. 6, 1968.

GERALD L. KAPLAN, Primary Examiner

U.S. Cl. X.R.

75—172; 204—47